

# UNITED STATES PATENT OFFICE.

TOMMASO PARZIALE, OF ALEXANDRIA, EGYPT.

## PROCESS OF MAKING SOAP.

SPECIFICATION forming part of Letters Patent No. 700,229, dated May 20, 1902.

Application filed August 18, 1900. Serial No. 27,336. (No specimens.)

*To all whom it may concern:*

Be it known that I, TOMMASO PARZIALE, a subject of the King of Italy, residing at Alexandria, Egypt, have invented certain new and useful Improvements in the Manufacture of Soap, of which the following is a specification.

This invention relates to the manufacture of soap having an oleaginous base, and in carrying out my invention into effect the quantity of cotton-seed oil it is desired to saponify is introduced into a zinc vessel and very fine flour containing gluten added in variable quantity. This quantity of flour may vary between ten and fifty per cent., according to requirements and with respect to the climate and the prevailing temperature in order to produce a larger development of ammonia-gas ( $NH_3$ ) for the saponification of the substances which the cotton-seed oil contains. This material renders the soap hygienic and economic. The source of the ammonia-gases is to be found in the chemical reaction between the nitrogenous matters of the flour and the caustic alkali. The mixture thus prepared cold is now left to stand for five to six hours. The purpose is to avoid the formation of small lumps. The rest after mixing serves to facilitate perfect amalgamation. Thereupon a solution is added of a caustic base or sodium hydrate, (soda of 30° Baumé,) about fifty per cent., by volume, and the mixture is thoroughly agitated. When furrows begin to show behind the beater, the mixture is placed in special boxes, in which it is left for three days, after which time it may be cut in the usual manner.

To the solution of caustic soda or sodium hydrate (formula  $NaOH$ ) may be added silicate of soda, alum, talc, cocoanut-oil, suitable perfume or essence, and the like, according to whether it is intended to prepare a cheap soap or one that is perfumed. There may be added silicate of soda or talc, besides other oils or essences, &c., according to whether cheaper soap has to be produced or

perfumed soap. This will facilitate the development of an ammoniacal gas. This proportion of talc and carbonate of lime may be from twenty to thirty per cent. If it is desired to obtain a soap as hard as that manufactured from olive-oil, twenty per cent. of silicate of soda is added.

It is immaterial whether the vessel is of iron or zinc.

The ammonia-gas is derived from the chemical reaction resulting from the combination of the nitrogenous matters (in floury condition) with the materials of the alkaline and caustic base, ( $NaOH$ .) To increase the development of this gas, it is only necessary to add to the nearly-condensed soapy mass two per cent. of a hot solution, consisting of one-half water and one-half alum in a well-mixed condition. As a consequence of this last addition and the reaction brought about thereby after about three days the soap has lost all its causticity, because the excess of hydrates has evaporated as gas, and thus a neutral soda oleate is obtained.

Zinc is the material of which the vessel is formed, since this metal is less liable to corrode through the action of the caustic alkali.

The mixture of oil and flour after having been worked in a cold state must rest from five to six hours, so that there may be brought about an absorption of those parts which are the most difficult ones to be absorbed—above all, the glycerin—in order to facilitate the reaction of the saponification.

I claim as my invention—

The process described consisting in mixing cold cotton-seed oil and flour containing gluten together, allowing the mixture to stand and then mixing with the said mixture caustic soda, substantially as described.

TOMMASO PARZIALE.

Witnesses:

EDUARD VAN DIEREN,  
EMILE CAPRARA.